

# UNITED STATES PATENT OFFICE.

RICHARD BUCK ARTHUR, OF BALLARAT, VICTORIA.

## PROCESS OF TREATING LEATHER.

SPECIFICATION forming part of Letters Patent No. 645,056, dated March 13, 1900.

Application filed August 30, 1899. Serial No. 728,990. (No specimens.)

To all whom it may concern:

Be it known that I, RICHARD BUCK ARTHUR, shopman, a subject of the Queen of Great Britain and Ireland, residing at 45 Nicholson 5 street, Ballarat, in the county of Grenville, Colony of Victoria, have invented a certain new and useful Process for Treating Leather and Similar Substances, of which the following is a specification.

10 The object of my invention is to render leather and similar substances unimpaired by contact with or immersion in water which is affected by minerals. In the past leather and like substances have suffered serious injury 15 under such circumstances; but with my process such materials, whether used for boots, shoes, harness, pumps, or any other purposes, are after treatment unaffected by the presence of water impregnated as above described.

20 My invention consists in first tanning the hide or skin or other substance in any ordinary way by chrome or bark or other tanning agencies and then suspending it in order that it may lose some of its moisture, after which, 25 if necessary, a split or shaving is removed, and it is then allowed to almost dry out. It is then placed in a rotating chamber or drum of any desired shape to absorb the first solution, which is composed as follows: Make a

30 mixture of five (5) pounds of alum, five (5) pounds of chalk, three (3) pounds of best glue, and about ten (10) gallons of water. The chamber is then set in motion and rotated for about four (4) hours or until the solution has thoroughly penetrated the substance, which is then removed and allowed to drain. After 35 draining it is hung up to almost dry out, when it is ready to receive the second solution, composed as follows: Dissolve ten (10) pounds of

40 pure asphaltum and one (1) pound of india-rubber in about three (3) gallons of turpentine, naphtha, or other solvent. Then add twelve (12) pounds of paraffin-wax and twelve (12) pounds of beeswax and four (4) pounds of 45 sugar of lead dissolved in oil. Reduce to the consistency required with boiled linseed-oil, paraffin-oil, or other oil. Have the whole thoroughly commingled by heating and agitation.

Previous to receiving the second solution

the chamber by steam, hot air, or other means 50 is heated to a temperature of about one hundred and thirty (130°) degrees Fahrenheit, provision being made, if steam is used, to drain out the accumulated water. After this the solution, which must also be heated to about 55 the same temperature, is placed with the leather or other substance in the chamber, which is then set in motion and run for about four (4) hours or for such shorter or longer period as will enable the solution to thoroughly permeate the leather. This is easily 60 determined by the practical tanner handling the leather. It is then removed from the chamber and, being set out in the usual way, is hung up to dry, after which it is finished 65 by the usual trade methods employed in finishing ordinary leather.

The quantities and times given above are approximate, since different descriptions of material require different proportions of the 70 above ingredients, which vary with the class of the leather and the purposes for which it is intended.

Having now described my invention, what I claim as new, and desire to secure by Letters 75 Patent, is—

An improved process for treating leather and similar substances consisting of tanning the leather in the ordinary way and then placing it in a rotating chamber containing a solution of alum, chalk, glue, and water in the approximate proportions specified, then draining and almost drying out, then placing it in a rotating chamber heated to a suitable temperature with a solution also heated as before 85 described consisting of asphaltum, india-rubber dissolved in turpentine or other solvent to which is added paraffin-wax, beeswax and sugar of lead dissolved in oil and of the approximate proportions specified, then finishing 90 in the ordinary way all as and for the purposes hereinbefore specified.

In witness whereof I have hereunto set my hand in presence of two witnesses.

RICHARD BUCK ARTHUR.

Witnesses:

WALTER JOSEPH NANSCAWEN,  
THOMAS HENRY JOHNSON.